

# UNITED STATES PATENT OFFICE.

JOSEPH ARMAND ERNEST HUBERT BOULLIER, OF PARIS, FRANCE.

## PROCESS FOR PRODUCING MANTLES FOR INCANDESCENT GAS-LIGHTING.

No. 844,849.

Specification of Letters Patent.

Patented Feb. 19, 1907.

Application filed March 23, 1903. Serial No. 149,199.

*To all whom it may concern:*

Be it known that I, JOSEPH ARMAND ERNEST HUBERT BOULLIER, a citizen of the Republic of France, residing at Paris, France, have invented Improvements in the Process for Producing Mantles for Incandescent Gas-Lighting, of which the following is a specification.

Many attempts have been made to produce incandescent gas-mantles from artificial silk and the like.

All the processes heretofore proposed have consisted in introducing incandescent compounds into a viscous solution of nitrocellulose capable of being spun into filaments, spinning the viscous mass into filaments, and then denitrating the same.

Nitrocellulose filaments are not penetrated by water, and they are therefore not adapted to fix incandescent compounds; but they acquire this property in a high degree when they are treated with liquids which are capable of causing them to swell without dissolving them. Certain acids—such as formic acid, acetic acid, and nitric acid in suitable degrees of concentration—possess this property.

The following table discloses the possible and preferred dilutions of such acids for use in my process:

|    | Possible proportions. | Preferred proportions.                             |
|----|-----------------------|----------------------------------------------------|
| 35 | 60 to 80.             | Acetic acid, (crystallizable),<br>$C_2H_4O_2$ . 75 |
|    | 40 to 20.             | Water, $H_2O$ . 25                                 |
|    | 35 to 50.             | Nitric acid, $HNO_3$ . 50                          |
|    | 65 to 50.             | Water, $H_2O$ . 50                                 |
|    | 90 to 100.            | Formic acid, $CH_3O_2$ . 100                       |
|    | 10 to 0.              | Water, $H_2O$ . 0                                  |

As appears from the above table, formic acid is used undiluted and at its maximum concentration. The same result may also be obtained by using alcohol mixed with a small quantity of commercial ether or with alcoholic ethers (ether salts) or with acetone and generally with any liquids or substances which alone or undiluted are capable of dissolving nitrocellulose. By reason of the presence of a liquid which has no dissolving action on nitrocellulose these mixtures may effect the swelling of the said filaments without dissolving them. The filaments thus physically modified are still nitrocellulose; but they have acquired the property of absorbing and even of fixing considerable quantities of incandescent salts.

In order to enable the nature of this invention to be clearly understood, the following example is given for the purpose of showing how it may be carried out. Nitric acid is selected as an example, because this acid is the cheapest; but the operation would be equally successful with concentrated formic acid of about ninety-five-per-cent. strength or with crystallizable acetic acid mixed with a small quantity of water. The degree of dilution of these acids may vary according to the temperature at which the operation is effected. The other liquids referred to hereinbefore may also be employed. It is to be understood that all the operations hereinafter described are equally applicable to nitrocellulose filaments as well as to knitted or woven fabrics made of these filaments.

The process is as follows:

First. The filaments of nitrocellulose are introduced into the diluted nitric acid of preferably 35° or 36° Baumé, and they are left to macerate in the acid until they have swelled up considerably. They have now become transparent or opaline and have a gelatinous appearance. Several hours are required in order to produce this result at ordinary atmospheric temperature; but the transformation is much more rapid at a temperature of about 35° Celsius. When the filaments have assumed the appearance above described, they are taken out of the acid, washed, and then treated in a centrifugal machine, and then they may be dried or not dried, as desired; but for the following operations it is preferable to employ the filaments in the moist state, so as not to diminish their absorbent capacity. This operation not only renders the filaments adapted to fix the incandescent salts, but also eliminates any mineral matters which may be contained in the nitrocellulose and which would injuriously affect the illuminating power or the strength of the filament.

Second. The nitrocellulose filaments thus modified are then immersed in a solution of, for instance, one hundred parts of commercial incandescent nitrates to one hundred parts of water. These proportions will vary according to the weight of the incandescent compounds which it is desired to fix in the filaments. After several hours of impregnation and even much less, especially if the operation is carried out with the application of heat, the filaments are taken out of the bath, then treated in a centrifugal machine

or squeezed for the purpose of eliminating therefrom the portion of the solution which has not become fixed. Then the filaments are left to dry at a gentle temperature.

5 Third. These filaments of nitrocellulose thus impregnated and dried are subjected to a denitrating process, such as the processes of denitration employed at present in the manufacture of artificial silk, but, by preference, to treatment with hydrated sulfate of ammonia, because it does not introduce into the filament any foreign substance which cannot be removed by washing with water.

15 The filaments produced by these operations are knitted or woven into mantles, or if the mantle itself has been treated the only remaining operation is to incinerate the mantle.

By this invention mantles may be produced

which will leave from thirty-five to forty per cent. of anhydrous oxids after combustion. They are strong, durable, and very luminous.

I claim as my invention—

The hereinbefore described method of manufacturing mantles for incandescent gas-lighting from nitrocellulose, said method consisting of first subjecting nitrocellulose filaments to a substance capable of causing said filaments to swell without dissolution and after thus causing them to swell, impregnating them with incandescing compounds.

Signed at Paris, France, this 7th day of March, 1903.

JOSEPH ARMAND ERNEST HUBERT BOULLIER.

Witnesses:

BENJAMIN BLOCHE,  
AUGUSTUS E. INGRAM.